

1,224,906.

H. H. DOEHLER.  
METHOD OR ART OF CASTING FLUID METALS.  
APPLICATION FILED SEPT. 10, 1915.

Patented May 8, 1917.



*Fig. 3.*



*Fig. 4.*



*Fig. 5.*



Attest:

John Doeher  
Judith Pardee

Heinrich H. Doeher Inventor:  
by Frank J. Wentworth  
his Atty.

# UNITED STATES PATENT OFFICE.

HERMAN H. DOEHLER, OF BROOKLYN, NEW YORK, ASSIGNOR TO DOEHLER DIE CASTING COMPANY, A CORPORATION OF NEW YORK.

## METHOD OR ART OF CASTING FLUID METALS.

1,224,906.

Specification of Letters Patent.

Patented May 8, 1917.

Application filed September 10, 1915. Serial No. 49,874.

*To all whom it may concern:*

Be it known that I, HERMAN H. DOEHLER, a citizen of the United States, residing at the borough of Brooklyn, city of New York, county of Kings, and State of New York, have invented certain new and useful Improvements in the Method or Art of Casting Fluid Metals, of which the following is a specification, reference being had therein to the accompanying drawings, which form a part thereof.

My invention relates to the method or art of casting fluid metals, and more particularly to a method or art wheréin the metal is forced and compacted, within a mold by means of fluid pressure.

In United States Letters Patent No. 973,483 granted to me under date of Oct. 25, 1910, I have described a method or art particularly adapted for use in casting metals having a high fusing point. The method or art, and the apparatus described in my aforesaid Letters Patent, have been extensively used in making commercial castings both of high fusing, and low fusing alloys.

In making castings of high fusing alloys, I have found it impracticable to make a large number of castings from a single metal mold, or die, because of the difficulties of introducing the molten metal to the apparatus in proper condition to secure a uniform run of commercially perfect castings. When the metal is melted in a furnace independent of the apparatus, and is delivered to the apparatus by means of a ladle, there is a tendency of the metal to lose sufficient heat through radiation to make it too sluggish to flow freely when entering the mold. To

40 avoid this condition, it was necessary to either maintain the mold at a sufficiently high temperature to compensate for the loss of heat by the molten metal; to raise the temperature of the molten metal above its fusing point in a degree which would prevent the loss of sufficient heat to interfere with the flow of the metal into all parts of the mold or die; or to use both these expedients.

50 Inasmuch as this method or art is used for producing castings, having a finished surface, and accurate as to dimensions, it is not only essential that the metal shall flow freely and not chill so rapidly when in the mold or die, as to cause surface imperfections or concealed blow holes, but that it

shall, after entering the mold or die, remain in condition for a sufficient interval to enable it to be compacted or compressed by the air or other fluid pressure applied to it as it is flowing under gravity into and after it 60 has entered the mold or die.

When the temperature of the mold was raised as above described, I found that I could use a high fusing alloy and produce commercially perfect castings, but that the 65 high temperature to which the mold or die was subjected not only had a tendency to rapidly warp the mold or die and prevent accuracy in the dimensions of the castings subsequently made therein, but to limit the 70 number of castings which could be produced from a mold or die, thus making it impracticable to produce castings in number and at a cost which made it commercially practical.

The heating of the metal materially above 75 its fusing point, had the disadvantage that it was not only injurious to the metal, but did not admit of uniformity in the product. Furthermore, when using the metal at very high temperatures, there was a tendency to 80 toward the warping of parts of small dimensions within the mold or die.

When both raising the mold or die to a high temperature, and raising the temperature of the metal well above its fusing point, 85 I found both of the disadvantages above referred to were present.

The conditions above referred to have not been present when practising the method or art, and using the apparatus of my aforesaid Letters Patent with white metal alloys, such having a lower fusing point than alloys rich in copper, or yellow alloys.

By means of the herein described improvements in the method or art described in my 95 aforesaid Letters Patent, I am enabled to make castings of high fusing alloys particularly those rich in copper, under conditions which avoid the maintenance of an excessively high temperature of the mold or die, or the raising of the temperature of the metal to be cast materially above its fusing point, thus permitting prolonged use of the mold or die and avoiding possible deterioration of the metal. I have made castings by 105 this method or art of a copper alloy having a fusing point of about two thousand degrees Fahrenheit with a mold or die used ordinarily for, and maintained under the same conditions ordinarily used in, casting 110

white metal alloys having a much lower fusing point; and these castings have been accurate as to measurements, have had a smooth, flawless surface, and have been free from superficial or concealed blow holes.

In the invention herein described, the manner of charging the mold or die is substantially the same as described in my aforesaid Letters Patent, this invention relating 10 more particularly to the specific manner of preparing each charge of metal, and of delivering it to the die or mold in such condition and in such volume as is necessary to produce one or more castings of the desired bulk together with that excess necessary to form a sprue.

My present invention has all the advantages of my patented invention when casting high fusing alloys with the additional 20 advantages that the mold or die is not required to be maintained at a temperature sufficiently high to warp the mold or die or make its handling in ejecting the casting slow; and that the alloy may be cast while 25 at substantially its fusing point.

The invention consists primarily in a method or art of casting fluid metals consisting of subjecting a melting pot or crucible containing metal of substantially the bulk of the casting to be made to a temperature approximating that of the fusing point of the metal, pouring the molten metal in said melting pot or crucible from within an inclosed chamber into a metal mold, and 35 thereafter forcing and compressing the metal by following it up with an elastic fluid under high pressure, and in such other novel steps and practice as are hereinafter set forth and described and more particularly pointed out in the claims hereto appended.

Referring to the drawings:

Figure 1 is a vertical section through an apparatus in which my method or art may 45 be practised;

Fig. 2 is a section on the line 2—2 of Fig. 1;

Fig. 3 is a perspective view of a conventional casting to be made;

50 Fig. 4 is a perspective view of an ingot of substantially the bulk of the casting shown in Fig. 3, and the sprue formed in making the casting, and

Fig. 5 is a vertical section of the melting 55 pot to be used with the ingot therein preparatory to its being melted.

Like letters refer to like parts throughout the several views.

In the practice of my improved method 60 or art, a metal alloy having a high fusing point is brought to and maintained at the desired or necessary temperature in a melting pot *a*. The alloy is illustrated in the accompanying drawings as being in the 65 form of an ingot *b* when placed in the melt-

ing pot, although it is apparent that this is not essential to the invention. The quantity of metal conditioned in the pot *a* is of substantially the same bulk as that of the casting or castings to be made therefrom, 70 and the sprue formed in making the casting.

The melting pot *a* with the molten metal therein is removed from the furnace in which it is subjected to heat at substantially 75 the temperature of the fusing point of the metal and placed within an inclosed chamber *c* from which it is poured into the mold or die *d* while still at a temperature of substantially that of the fusing point of the 80 alloy. Leading from the chamber *c* to the mold *d* is an ingate opening *e* which is constricted adjacent the mold and extended adjacent the chamber *c* to form a sub-chamber *c'* at the bottom thereof. This ingate extends substantially vertically so as to cause the molten metal to have a tendency to flow under gravity from the chamber *c* into the mold.

The chamber *c* is adapted to be opened to 90 permit the insertion of the melting pot *a* therein, and the mold or die *d* is made in a plurality of parts to permit the drawing or ejection of the casting. The melting pot *a* is provided with a suitable handle *a'* by 95 which it may be handled and operated.

The chamber *c* having been closed after the mounting of the melting pot *a* therein, the melting pot is overturned and the molten metal contained therein is poured into the 100 bottom of the chamber *c* and the sub-chamber *c'* from whence it will begin to flow under gravity through the ingate *e* into the mold. The constricted passage between the chamber *c* and the mold or die *d* formed by 105 the said sub-chamber and the said ingate will collect and concentrate the molten metal.

Immediately after, or substantially simultaneously with the pouring of the metal from within the chamber *c*, air or other suitable fluid, under pressure, is admitted to the chamber *c* through the valve controlled pipe line *f*, the pressure being determined by the size or character of the casting to be made. The discharge of the air line *f* is so positioned as to prevent a fluid jet impinging upon the molten metal in a manner to splash the same about said chamber.

It will be observed that there is an equilibrium of pressures in the chamber *c* and mold or die *d* when pouring the metal from the melting pot *a*, and that the admission of fluid pressure to the chamber *c*, destroys this equilibrium while there is a barrier of molten metal between said chamber and the mold or die, with the preponderating pressure within the chamber *c*.

This condition accelerates the rate of flow of the molten metal, converting the entire 130

charge into a metallic ram as it enters the mold and forcing it into all parts thereof, filling all cavities and interstices instantaneously. Incidentally, as the metal enters the 5 mold or die, it is compressed or compacted in a manner to avoid any concealed blow holes, the fluid under pressure being excluded from the mold or die by the metal passing through the ingate.

10 The metal sets or solidifies substantially simultaneously with its contact with the walls of the mold, retaining sufficient fluidity, however, toward the center and top of the casting to admit of the compression or 15 compaction above referred to.

While there is a tendency of the metal to chill and adhere to the wall of the ingate *e*, this does not interfere with the flow of the metal to an extent to prevent the desired 20 rapid charging of the metal into the mold or die. It does, however, form a substantial sprue, and must be taken into account in determining the bulk of metal to be conditioned in the melting pot *a*.

25 The chamber *c* is vented before the mold or die is opened to permit the drawing of the casting.

When referring to the "conditioning" of the metal, herein, I have reference merely 30 to the bringing of the metal to, or its maintenance at, a temperature of, or slightly above, the fusing point thereof while in the melting pot from which it is poured.

While I have made satisfactory castings 35 in an ordinary steel die, such as is used for making castings of lower fusing alloys than those to be cast by the method or art herein described, it is apparent that this invention is entirely independent of the material or 40 construction of the die and the particular apparatus by means of which it is practised.

The essential and dominating characteristics of the invention herein described, as 45 compared with my aforesaid patented method or art, are that a charge approximating in bulk, the mass of metal required for a single casting, is brought to the desired or necessary temperature while in a melting 50 pot, and that the charge is poured directly from said melting pot, as a ladle, into the mold or die under the conditions herein specified. These characteristics, I have found, prevent a loss of sufficient heat to prevent 55 the metal flowing freely from the pressure chamber into the mold, and permit the casting of a metal having a high fusing point, while at a temperature substantially that of the said fusing point and without raising the 60 temperature of the mold above normal.

I have not described in detail the apparatus shown in the accompanying drawings, as that is made the subject of a separate application.

65 The condition or form in which the metal

is placed in the melting pot is immaterial so long as the bulk of such metal is sufficient only for a single casting operation, and so long as the melting pot and the metal therein are subjected to a temperature of substantially the fusing point of the alloy used just prior to such casting operation. 70

While I have referred to an alloy having a fusing point of about two thousand degrees Fahrenheit, my method or art may 75 be practised in making castings of an alloy the fusing point of which may be above or below this temperature.

Having described the invention, what I claim as new and desire to have practised by 80 Letters Patent, is:—

1. The herein described method or art of casting fluid metal, consisting of subjecting a melting pot or crucible containing metal of substantially the bulk of the casting to be 85 made to a temperature approximating that of the fusing point of the metal until the metal is reduced to a molten condition, pouring the molten metal in said melting pot or crucible from within an inclosed 90 chamber into a metal mold, and thereafter forcing and compressing the metal by following it up with an elastic fluid under high pressure.

2. The herein described method or art of 95 casting fluid metal, consisting of subjecting a melting pot or crucible containing metal of substantially the bulk of the casting to be made to a temperature approximating that of the fusing point of the metal until the 100 metal is reduced to a molten condition, pouring the molten metal in said melting pot or crucible from within an inclosed chamber into a metal mold, and subjecting it while it is flowing from said chamber to the mold. 105 to an elastic fluid under high pressure.

3. The herein described method or art of casting fluid metal, consisting of subjecting a melting pot or crucible containing metal of substantially the bulk of the casting to 110 be made to a temperature approximating that of the fusing point of the metal until the metal is reduced to a molten condition, pouring the molten metal in said melting pot or crucible from within an inclosed chamber into a constricted passageway leading to a metal mold, and forcing and compressing the metal by subjecting it while it is flowing through said passage way to an elastic fluid under high pressure. 115

4. The herein described method or art of casting fluid metal, consisting of subjecting a melting pot or crucible containing metal of substantially the bulk of the casting to be made to a temperature approximating 125 that of the fusing point of the metal until the metal is reduced to a molten condition, pouring the molten metal in said melting pot or crucible from within an inclosed chamber into a metal mold, maintaining an

equilibrium of pressures within said chamber and said mold while pouring, and destroying the equilibrium of pressures with a predominating pressure within said inclosed chamber whereby while the metal is flowing to the mold by gravity its movement is accelerated and it is forced into and compressed in the mold under heavy pressure.

5. The herein described method or art of casting fluid metal consisting of subjecting a melting pot or crucible containing metal of substantially the bulk of the casting to be made to a temperature approximating that of the fusing point of the metal until the metal is reduced to a molten condition, pouring the molten metal in said melting pot or crucible from within an inclosed chamber into a constricted passage way leading to a metal mold, maintaining an equilibrium of pressures within said chamber and said mold while pouring, and destroying the equilibrium of pressures with a preponderating pressure within said inclosed chamber, whereby while the metal is flowing to the mold by gravity its movement is accelerated and it is forced into and compressed in the mold under heavy pressure.

6. The herein described method or art of casting fluid metal consisting of subjecting a melting pot or crucible containing metal of substantially the bulk of the casting to be made to a temperature approximating that of the fusing point of the metal until the metal is reduced to a molten condition, pouring the molten metal in said melting pot or crucible from within an inclosed chamber into a metal mold, and forcing and compressing the metal by subjecting it while it is flowing from said chamber into the mold to the expansion of an elastic fluid under high pressure.

7. The herein described method or art of casting fluid metal, consisting of subjecting a melting pot or crucible containing metal of substantially the bulk of the casting to be made to a temperature approximating that of the fusing point of the metal until the metal is reduced to a molten condition, pouring the molten metal in said melting pot or crucible from within an inclosed chamber into a constricted passage way leading to a metal mold, and forcing and compressing the metal by subjecting it while it is flowing through said constricted passage way to the expansion of an elastic fluid under high pressure.

8. The herein described method or art of casting fluid metal consisting of subjecting a melting pot or crucible containing metal of substantially the bulk of the casting to be made to a temperature approximating that of the fusing point of the metal until the metal is reduced to a molten condition,

pouring the molten metal in said melting pot or crucible from within an inclosed chamber into a metal mold, maintaining an equilibrium of pressures within said chamber and said mold while pouring, and destroying the equilibrium of pressures with a preponderating pressure within said inclosed chamber, whereby while the metal is flowing to the mold by gravity its movement is accelerated and it is forced into and compressed in the mold under heavy pressure.

9. The herein described method or art of casting fluid metal consisting of subjecting a melting pot or crucible containing metal of substantially the bulk of the casting to be made to a temperature approximating that of the fusing point of the metal until the metal is reduced to a molten condition, pouring the molten metal in said melting pot or crucible from within an inclosed chamber into a constricted passage way leading to a metal mold, maintaining an equilibrium of pressures within said chamber, said passage way and said mold while pouring, and destroying the equilibrium of pressures with a preponderating pressure within said inclosed chamber by the expansion of an elastic fluid under high pressure, whereby while the metal is flowing by gravity its movement is accelerated and it is forced into and compressed in the mold under heavy pressure.

10. The herein described method or art of casting fluid metal consisting of subjecting a melting pot or crucible containing metal of substantially the bulk of the casting to be made to a temperature approximating that of the fusing point of the metal until the metal is reduced to a molten condition, pouring the molten metal in said melting pot, or crucible from within an inclosed chamber into a mold maintained at a temperature below the fusing point of said metal, through a constricted passage way, having an enlarged portion at said chamber, and delivering a fluid under high pressure to said inclosed chamber immediately after pouring said metal from said melting pot or crucible whereby while the metal is flowing by gravity, its movement is accelerated and it is forced into and compressed in the mold under heavy pressure.

In witness whereof I have hereunto affixed my signature in the presence of two subscribing witnesses, this 1st day of September, 1915.

HERMAN H. DOEHLER.

Witnesses:

F. T. WENTWORTH,  
A. S. HUNKEL.